

## UNITED STATES PATENT OFFICE

HORACE CAMPBELL HALL AND TENNYSON FRASER BRADBURY, OF DERBY, ENGLAND,  
ASSIGNORS TO ROLLS-ROYCE LIMITED, OF DERBY, ENGLAND

## ALUMINUM ALLOY

No Drawing. Application filed October 23, 1929, Serial No. 401,870, and in Great Britain December 18, 1928.

The object of this invention is to make an aluminum alloy having certain properties superior to those of any aluminum alloys heretofore known.

5 It is common knowledge that aluminum alloys often undergo an appreciable decrease in strength and hardness when subjected to an increase of temperature. In aluminum alloys where an improvement in characteristics takes place by heat treatment it is frequently found that an impairment of the characteristics takes place when the alloy is subsequently heated to a moderate temperature, although in some cases and under 10 some conditions, the deterioration is reduced or the former condition restored on a return to normal temperature. Our invention has for its object to overcome or reduce the disadvantages and deterioration before mentioned.

20 An alloy made according to this invention is one improved by heat treatment, and which is affected to a very small extent by subsequent heating to a moderate temperature.

25 According to this invention we make an alloy by compounding the elements, and that in relative quantities within the ranges set out below:—copper 0.5 to 5.0 per cent of the whole, magnesium 0.1 to 1.7 per cent of the whole, nickel 0.2 to 1.5 per cent of the whole, iron 0.6 to 1.5 per cent of the whole, silicon 30 .55 to 2.8 per cent of the whole, titanium up to .3 per cent of the whole, manganese up to .3 per cent of the whole, aluminum the remainder, only traces of other elements.

35 With an alloy compounded as above, a casting can be made which is light, strong, easily and satisfactorily cast and forged, gives good resistance to corrosion and possesses good mechanical qualities. Further the castings and forgings are susceptible to both high and low temperature in heat treatment to give improved mechanical properties.

40 Further, an alloy according to this invention is less susceptible to the harmful effects of vibration and fatigue than are known alloys.

45 As an example of this alloy with the magnesium content about 1.5 per cent and the copper about 2.5 per cent the strength and

hardness are less affected on re-heating to about 300° C. than with known alloys and are restored on re-cooling. Such an alloy would be very suitable for such parts as pistons and connecting rods.

55 With an intricate casting or with one which was to be forged subsequently or heat treated, or both, some departure from that composition would be necessary.

60 If a very light alloy were required the proportions of both magnesium and silicon should be at the high end of the ranges with possibly a small sacrifice in physical properties or casting facilities or both.

65 The alloy is made in manner common in foundry practice, that is to say, to molten commercial aluminum, we add aluminum alloys each rich in one or in some cases more than one of the required elements.

70 What we claim is:—

An aluminum alloy formed by compounding the elements, and that in relative quantities respectively within the ranges set out below:—copper 0.5 to 5.0 per cent of the whole, magnesium 0.1 to 1.7 per cent of the whole, nickel 0.2 to 1.5 per cent of the whole, iron 0.6 to 1.5 per cent of the whole, silicon .55 to 2.8 per cent of the whole, titanium up to .3 per cent of the whole, manganese up to .3 per cent of the whole, aluminum the remainder, only traces of other elements.

75 In testimony whereof we have affixed our signatures.

HORACE CAMPBELL HALL.  
TENNYSON FRASER BRADBURY.

85

90

95

100